

[54] METHOD FOR STRENGTHENING A METAL SURFACE

164/105, 106, 107, 319, 321, 97

[75] Inventors: Yoshifumi Sakai, Chiryu; Takeshi Sumi, Chita; Atsushi Wada, Tokai; Mitsuo Morishima, Tokai; Shigeto Kawakaki, Tokai; Takashi Kozawa, Nagoya, all of Japan

[73] Assignee: Daido Deiko Kabushiki Kaisha, Aichi-ken, Japan

[22] Filed: Dec. 22, 1971

[21] Appl. No.: 210,733

[30] Foreign Application Priority Data  
Dec. 29, 1970 Japan 45/121220

[52] U.S. Cl. 164/59, 164/98, 164/120  
[51] Int. Cl. B22d 19/00, B22d 27/18

[58] Field of Search. 164/59, 75, 120, 98, 100, 103,

[56]

References Cited

UNITED STATES PATENTS

2,161,597 6/1939 Swartz ..... 164/75 X  
2,034,550 3/1936 Adams ..... 164/98 X

FOREIGN PATENTS OR APPLICATIONS

431,372 1/1968 Japan ..... 164/97

Primary Examiner—J. Spencer Overholser  
Assistant Examiner—John E. Roethel

[57]

ABSTRACT

A metal surface strengthening method comprising attaching, with or without pressure, a preformed plate formed of a metal surface strengthening powder to a fundamental molten metal kept in a gas sprayed protective atmosphere in the mold.

2 Claims, 7 Drawing Figures



PATENTED FEB 19 1974

3,792,726

SHEET 1 OF 2



FIG. 1



FIG. 4



FIG. 2



FIG. 5



FIG. 6

PATENTED FEB 19 1974

3,792,726

SHEET 2 OF 2



FIG. 3



FIG. 7

# METHOD FOR STRENGTHENING A METAL SURFACE

## BACKGROUND OF THE INVENTION

Hitherto, case hardening, nitriding, spraying, plating, welding, etc., have widely been utilized as metal surface strengthening methods. Recently, however, a method in which metal surface strengthening is carried out in the course of molten metal squeeze casting is under development (e.g., Japanese Pat. No. 520,699). This method is concerned with an applied technique of squeeze casting, wherein the metal surface strengthening powder is directly scattered on wherein molten metal poured in the mold, and the pressure is subsequently applied thereto to form a strengthened metal layer. This method enables one to obtain the desired strengthened metal layer simultaneously with the completion of the product, and so is a method to be highly appreciated. At present, however, this method has drawbacks as mentioned below:

1. Since the molten metal surface in the mold is in an oxidized state at the time the powder is scattered thereon, the reaction between the powder and the molten metal becomes incomplete so that even if the pressure is sufficiently applied thereto, the resulting product often tends to tear off at the bonded portion.

2. Furthermore, as the powder, when scattered on the molten surface, is heated by the molten metal and is oxidized by oxygen in the air, it may lose its metal strengthening nature. For example, if the powder is of WC (tungsten carbide), W in the WC reacts with O<sub>2</sub> so that the resulting layer is not sufficiently strengthened.

Because of these disadvantages, it has been difficult, as shown in FIGS. 1 and 2, to form products with smooth casting surfaces and uniform strengthened layers (A).

## SUMMARY OF INVENTION

This invention relates to a method for strengthening a metal surface comprising the steps of pouring a molten metal into a mold, placing or laying a preformed plate compacted from a mixture of one or more of a powder of tungsten carbide, titanium carbide, tantalum carbide and ceramic and a powder of a binder on the surface of said molten metal, and applying pressure by means of a punch during the molten state or solidification course of said molten metal so that said plate is directly bonded to the surface of said metal whereby a strengthening layer is formed on the surface of said metal.

This invention aims at removing the defects mentioned hereinbefore, permitting strengthening of the metal surface by a relatively simple method, and further, permitting industrial mass production for the method.

## BRIEF DESCRIPTION OF THE DRAWINGS

FIG. 1 is a photomicrograph ( $\times \frac{1}{2}$ ) showing the casting surface of a strengthened layer made in accordance with a conventional powder scattering method;

FIG. 2 is a photomicrograph ( $\times \frac{1}{2}$ ) representing a cross sectional view of the thickness distribution of a metal layer strengthened in accordance with the conventional powder scattering method;

FIG. 3 is a cross sectional view of one embodiment of this invention; and

FIGS. 4 - 7 are photomicrographs and a diagram of the embodiments effected in accordance with the present invention, wherein FIG. 4 is a photomicrograph ( $\times \frac{1}{2}$ ) of the casting surface of a strengthened layer; FIG. 5 is a photomicrograph ( $\times \frac{1}{2}$ ) of a section of the thickness distribution of a strengthened layer; FIG. 6 is a photomicrograph ( $\times 100$ ) of the microstructure of the bonded part of a strengthened layer with a fundamental material; and FIG. 7 is a diagram of the distribution of hardness (H<sub>v</sub>) of the strengthened layer shown in FIG. 6.

## DESCRIPTION OF PREFERRED EMBODIMENTS

The method of this invention will now be explained with reference to FIG. 3 of the accompanying drawings.

The preformed plate is formed to one 5 mm thick piece from a mixture 1a of the powder comprising at least 90 percent of one or more of tungsten carbide, titanium carbide, tantalum carbide, ceramics, etc., each having a good affinity with the molten metal, and approximately 10 percent of a binder such as a thermosetting resin, on an asbestos adiabatic sheet 1b producing no slag when reacted with the molten metal.

A desired molten metal 3 is then poured into the mold 2 which is sprayed with a wash for accomplishing a releasing action at the inside wall of said mold, when the atmosphere in the mold 2 is kept non-oxidized protective to prevent the molten metal 3 from oxidizing. For this purpose, the nozzles 7 provided at the upper inside of the mold 2 are connected to the protective gas supplying pipe 6. The preformed plate 1 is then placed or laid on the surface of the molten metal 3, and after a lapse of a proper time (e.g., about 10 sec.) a pressure punch 4 is lowered to apply thereto an amount of pressure (e.g., about 1 ton/cm<sup>2</sup>; about 30 sec.). Thereafter, the pressure is released and the product of a predetermined shape is taken out by means of a knockout pin 5.

FIG. 4 shows a casting surface of a strengthened surface formed according to the method of this invention and FIG. 5 illustrates a strengthened layer (B) formed by the method of this invention. It has been found that both of them have the merits as mentioned hereinafter in comparison with the conventional scattering method. As is clear from the comparison of FIG. 1 with FIG. 4, the casting surface is superior in the case of the present invention. For instance, the shortcomings such as blow holes, tearing off of the strengthened layer, etc., that have often taken place with the prior method have been remarkably decreased. A comparison of the reference numeral A of FIG. 2 with the reference numeral B of FIG. 5 clearly shows that the strengthened layer with a uniform and desired thickness as shown in FIG. 5 can also be obtained by the method of the present invention.

Furthermore, in the product obtained by the method of this invention, the strengthened layer is so firmly bonded to the molten metal due to the application of pressure by means of the punch 4 that, when used for a punching die and the like requiring a substantial hardness and a toughness, such undesirable phenomena as half-wearing, lacking, and tearing-off in the case of the conventional die do not occur so that a remarkable effect results in that the life span of the product is prolonged.

FIG. 6 represents the microstructure ( $\times 100$ ) of the bonded part of the strengthened layer to the fundamental material obtained by the method of the present invention. This test material has been prepared by bonding to the molten metal of carbon steel a preformed plate formed of WC (tungsten carbide) powder, said test material having been subjected to an annealing process thereafter. From this figure, it can be seen that the attachment near the boundary portion (C) is perfect and no noxious defects such as an inclusion or gas effect are recognized.

FIG. 7 is a diagram showing the distribution of Vickers hardness (Hv) extending from the strengthened layer as shown in the photomicrograph of FIG. 6 to the fundamental material. As is clear from the diagram, the strengthened layer (made from tungsten carbide) remains sufficiently strengthened after it has been annealed.

As described above in detail, it has been shown that the method of the present invention is far superior to that of the conventional powder scattering method. For instance, in case a strengthened layer is to be attached to an uneven metal surface, it has been very difficult to attach it uniformly due to the fluidity of the molten metal. According to this invention, however, a preformed plate formed to any desired shape from the powder for strengthening a metal surface is placed or laid on the molten metal in the mold or core mold so that products with evenly strengthened surfaces can be obtained.

According to the present invention, as described above, the metal surface strengthening can be carried out by the relatively simple method. Moreover, various composite materials in the fields of wearing, heat, and erosion resistance industries can be manufactured at remarkably low costs. Also, the object of using the preformed plate in this invention is that the operation can be carried out effectively and a smoothed casting surface and uniform thickness of strengthened layer can be obtained. Furthermore, in case the features of the molten metal and those of the powder for strengthening are quite different thereby making the attachment therebetween difficult, they can be attached by adding to the preformed plate one or more layers of materials required for their attachment.

What is claimed is:

1. A method for strengthening a metal surface comprising the steps of pouring a molten metal into a mold, placing a preformed plate compacted from a mixture of one or more of a powder of tungsten carbide, titanium carbide, tantalum carbide and ceramics and a powder of a binder on the surface of said molten metal, and applying pressure by means of a punch during the molten state of said molten metal so that said plate is directly bonded to the surface of said metal whereby a strengthened layer is formed on the surface of said metal.
2. The method of claim 1 wherein the pressure is applied during the solidification of said molten metal.

30

\* \* \* \* \*

35

40

45

50

55

60

65

UNITED STATES PATENT OFFICE  
CERTIFICATE OF CORRECTION

Patent No. 3,792,726 Dated February 19, 1974

Inventor(s) Yoshifumi Sakai, Takeshi Sumi, et al

It is certified that error appears in the above-identified patent and that said Letters Patent are hereby corrected as shown below:

On the first page, column 1, line 8, the Assignee's name should read --Daido Seiko-- instead of "Daido Deiko"

Signed and sealed this 13th day of August 1974.

(SEAL)

Attest:

McCOY M. GIBSON, JR.  
Attesting Officer

C. MARSHALL DANN  
Commissioner of Patents